

Patented Apr. 18, 1933

1,903,842

# UNITED STATES PATENT OFFICE

COURT C. TITUS, OF NEW YORK, N. Y.

## ALUMINUM ALLOY

No Drawing.

Application filed May 20, 1932. Serial No. 612,651.

My invention relates to a series of aluminum alloys of novel composition and properties. The alloys of my invention are particularly characterized by the presence of boron and magnesium and by the absence of substantial amounts of silicon, copper and iron. The presence of one or more metals of the group comprising vanadium, tungsten, molybdenum, chromium and cobalt, is also characteristic of the preferred form of my new alloys.

The alloys of the invention combine light weight with a high hardness and tensile strength. A surprising property of the new alloys is their high electrical conductivity and resistance to corrosion.

The metals may be utilized either in the cast condition, or they may be rolled, drawn or otherwise worked. Mechanical working is preferably carried out at a temperature of 150°-450° C. and such working effects a material increase in the tensile strength of the alloys. Wire drawn from the alloys of the invention is particularly valuable, since it combines a relatively high tensile strength with a relatively high conductivity. A further valuable property of such wires is that sleet and snow do not readily stick to them.

A particularly valuable alloy embodying my invention has the following composition:

|           |           |
|-----------|-----------|
| Magnesium | 1.25%     |
| Boron     | 0.75%     |
| Vanadium  | 0.75%     |
| Tungsten  | 0.75%     |
| Aluminum  | remainder |

The amount of magnesium may vary from about 0.25% to about 2.25%, the preferred amount being from 0.75% to 1.5% and the boron from 0.05% to 2%, although at least 0.25% is preferable and in many cases it is preferable not to add over 0.75% of boron due to the increased brittleness caused by higher amounts. Either vanadium or tungsten may be used alone in these alloys, and either or both may be replaced in whole or in part by one or more of the metals molybdenum, chromium and cobalt. In general it is advantageous to use the metals of the

group including vanadium, tungsten, molybdenum, chromium and cobalt in amounts of from 0.25% to 3.0%; larger amounts may be used, but they tend to increase the specific gravity and the cost of the alloy.

In general it may be said that a principal function of boron in the alloys of the invention is to increase the hardness; a principal function of the magnesium is to decrease the specific gravity and increase the resistance of the alloys against corrosion; and the principal function of the tungsten, vanadium, molybdenum, cobalt and chromium is to increase the tensile strength of the alloys.

Alloys of the invention as described above have been obtained having a specific gravity of 2.66 to 2.70; a tensile strength when cast of 30,000 to 41,000 pounds per square inch, and when mechanically worked of from 51,000 to 56,000 pounds; and an electrical conductivity of 50-58 (Ag=100).

An advantageous method of producing the alloys of the invention is as follows: The aluminum is melted in a crucible and covered with a layer of powdered charcoal. The charcoal serves to protect the metal from oxidation and to reduce those metals which are added in the form of oxides. The magnesium is added as metal and the boron, tungsten and vanadium or their substituting metals as oxides. The added metals or their oxides are advantageously added enclosed in aluminum capsules. The boron oxide is preferably added first, although it may be added together with the magnesium. The other metal oxides may be added together.

I claim:

1. An alloy consisting principally of aluminum and containing from 0.05 to 2% of boron, from 0.25 to 2.25% of magnesium, and from 0.25 to 3% of at least one metal of the group consisting of vanadium, tungsten, molybdenum and chromium.

2. An alloy consisting principally of aluminum and containing from 0.25 to 0.75% of boron, from 0.75 to 1.5% of magnesium, and from 0.25% to 3% of at least one metal of the group consisting of vanadium, tungsten, molybdenum and chromium.

3. An alloy of about the following composition:

|            |       |
|------------|-------|
| Magnesium  | 1.25% |
| Boron      | 0.75% |
| 5 Vanadium | 0.75% |
| Tungsten   | 0.75% |

and the remainder principally aluminum.

4. An alloy consisting principally of aluminum and containing from 0.05 to 2% of boron, from 0.25 to 2.25% of magnesium and from 0.25% to 3% of vanadium.

In testimony whereof, I affix my signature.

COURT C. TITUS.

15

20

25

30

35

40

45

50

55

60